

Aug. 3, 1926.

1,594,344

H. E. BAKKEN

PRODUCTION OF MAGNESIUM

Original Filed Nov. 1, 1922 2 Sheets-Sheet 1



Fig. 1.

Inventor

*H.E. Bakken*

By *John Boyle Jr.*  
Attorney.

Aug. 3, 1926.

1,594,344

H. E. BAKKEN

PRODUCTION OF MAGNESIUM

Original Filed Nov. 1, 1922 2 Sheets-Sheet 2



Fig. 3.



Fig. 4.



Fig. 2.

Inventor

H.E.Bakken

By *John Boyle*  
Attorney

## UNITED STATES PATENT OFFICE.

HERMAN E. BAKKEN, OF NIAGARA FALLS, NEW YORK, ASSIGNOR TO AMERICAN MAGNESIUM CORPORATION, OF NIAGARA FALLS, NEW YORK, A CORPORATION OF NEW YORK.

## PRODUCTION OF MAGNESIUM.

Application filed November 1, 1922, Serial No. 598,292. Renewed April 17, 1926.

My invention relates to the production of metallic magnesium in a substantially chemically pure state. By the processes that are at present practiced, magnesium when produced from ores containing other metals and metalloids, is likely to be contaminated with them. For use in the mechanical arts, these impurities must be removed as it is found that they exert a marked influence on the physical and chemical properties of the metal when present in only a very limited degree.

My process is particularly adapted for use in refining crude metal. It is applicable also to obtaining pure metal from magnesium scrap, such as castings, alloys, etc.

My invention comprises the purification of magnesium by converting the solid metal directly into the state of vapor and then condensing it directly in the solid state without intermediate liquefaction, and in particular it consists in the discovery of suitable means and conditions whereby such purification can be made practically operable and capable of being commercially carried out so as to produce pure magnesium at a reasonable cost.

It is known that magnesium boils at atmospheric pressure at about 1120° C. Purification by distillation at this temperature, however, is in practice very difficult because of the fact that the necessary apparatus deteriorates rapidly at such a high temperature. By reducing the pressure in the apparatus, i. e. by carrying on the distillation under diminished pressure, the boiling point of the metal can be reduced, until it coincides with the melting point at a pressure of approximately 2 millimeters of mercury, thus reducing the difficulty found in producing a suitable apparatus of a sufficient size to handle commercial quantities of metal, and strong enough to satisfactorily withstand the continued external pressure involved.

I have discovered, however, that if the pressure inside the apparatus is still further reduced, say to less than about 1 mm., rapid sublimation of the magnesium may be accomplished at temperatures which are within the range where ordinary steel apparatus will function satisfactorily. In order to obtain rapid sublimation, it is necessary to so adjust or regulate the operating pressure to a point where the total absolute pressure

in the condenser is slightly less than the vapor pressure of the magnesium at the temperature of the solid metal being sublimed. Under these conditions, the evolution of magnesium vapor will be rapid and if proper condensation facilities are provided the rate of sublimation is only limited by the rate at which heat can be supplied to the metal being sublimed. This point at which the vapor pressure of the solid magnesium becomes greater than the absolute pressure of the system is hereinafter called the "sublimation point".

By virtue of operating at or above the sublimation point I do not only produce rapid sublimation, but by the rush of magnesium vapor toward the condenser I sweep out and away the residual amount of air or other gas in the apparatus, and thus reduce very much the tendency of this gas to combine with the magnesium and render the product impure.

One of the great advantages of my method of sublimation as compared with vacuum distillation of magnesium is that not only can it be made to be as rapid as the distillation but it also gives a considerably purer product. In vacuum distillation I have found that no matter how carefully the distillation is carried on, there is always a certain proportion of non-volatile or substantially non-volatile impurities, carried over into the condensed metal. I ascribe this phenomenon to the well-known tendency of gases or vapors to carry with them minute droplets or spray of any liquid thru which they pass or from which they are evolved, particularly if they are evolved rapidly. This spray of impure magnesium carried over from the boiling liquid contaminates the distillate, but its formation appears to be prevented by subliming rather than distilling the magnesium so as to avoid the phenomenon of the evolution of bubbles from a liquid.

It will be apprehended that the process is capable of being carried out in a number of different types of apparatus and that the one shown and described is merely illustrative of the principles of the invention. This embodiment, however, has been found to be practical in construction and operation and efficient in use.

Referring to the drawings for a more complete disclosure of the invention:

Figure 1 is a vertical longitudinal section of the furnace;

5 Figure 2 is a section on the line 2—2 of Figure 1;

Figure 3 is a detail of the cover and closing mechanism for the retort;

10 Figure 4 is a section on the line 4—4 of Figure 1;

The iron retort 1 is suitably supported and inclosed in a brickwork and may be heated by burners projecting through the openings 2 and 3 in the lower corners of the combustion chamber, or in any other suitable manner. The retort at its lower ends is supported by the vertical brick wall 5 and by the wall collar 6. Intermediate its ends, it is supported by a wall collar 7 carried by the 15 center wall 8 and at its front end by the wall collar 9 carried by the front wall 10. In such a construction, the greater part of the retort is in the zone of heat, the remainder extending out into the air to provide a cold end therefor, which may be provided with cooling coils.

15 The charging end of the retort is closed by a suitable door 11 which is so constructed as to make the same as gas tight as possible. A suitable construction comprises lugs 13 integral with the retort and a series of hooks 20 welded to the lugs and clamped between the bars 14 of the framework 15. Carried between the said bars are 20 screw blocks 16 which engage with the screws 17 of the hand wheels 18. Rotation of the said wheels in suitable direction will loosen or tighten the cover of the retort.

25 For determining the temperature at the bottom of the retort a pyrometer well 19 is provided and a similar pyrometer well 21 is provided at the top of the retort.

30 For facilitating removal of the deposited crystals a liner 22 is located in the cooler end of the retort.

35 This liner consists of a pipe somewhat smaller than the inside diameter of the retort, so that it can be easily slipped in and taken out. The liner is open at both ends, and at its lower end rests on the annular ring 23, integral with the pot, the other end extending up to the closing flange. The purpose of the ring 23 is to keep the liner from slipping down into the retort and also 40 to form a seal so that gaseous magnesium does not travel up between the liner and the retort wall. The liner may be made in one piece or split longitudinally into two halves, to facilitate removal of the deposited crystals.

#### Operation.

45 The pot is charged with a suitable quantity of crude, impure, or alloyed magnesium, sealed and vacuum applied. When the

manometer shows the desired degree of vacuum has been obtained, heat is applied, care being taken to maintain the vacuum. After a suitable period of time, the temperature will rise to about 600 degrees C. and 70 is held there for about 5 or 6 hours. At the end of that time, the source of heat is cut off and the retort allowed to cool while still under the same vacuum.

75 Under the conditions outlined, the magnesium does not melt but passes directly from the solid into the vapor state. The vapor passes into the cooler portion of the retort where it condenses on the liner. When opened, the inner surface of the liner will 80 be found to be covered with crystallized magnesium which can be removed in a suitable manner. Analysis of the residue in the bottom of the retort will show that nearly all the magnesium has been vaporized. Analysis of the crystals of magnesium 85 will show that the magnesium content may be as high as 99.989%.

90 The best available data indicate that the vapor pressure of magnesium decreases from one atmosphere or 760 mm. of mercury at 1120° C., which is ordinarily spoken of as its boiling point, to approximately 2 mm. at its melting point, 651° C. Below the melting point the vapor pressure gradually decreases, so that after a further drop of about 270° C. it is still about 0.001 mm. If crude, impure or alloyed magnesium is heated at a 95 temperature below its melting point, the magnesium will vaporize so as to produce a partial pressure of magnesium vapor, determined by the temperature. If this heating is done in the presence of an inert gas such as argon, at atmospheric pressure or 100 under diminished pressure, but still at a total pressure greater than the vapor pressure of magnesium at the temperature employed, this magnesium vapor will diffuse thru the inert gas; and if another part of the apparatus is cooler than the metal being 105 heated, magnesium will gradually condense 110 in this portion of the apparatus. This rate of sublimation is so slow, however, that I have found it very advantageous to reduce the total pressure within the condenser to a 115 point below the vapor pressure of the magnesium at the temperature employed, as measured at 19, Fig. 1. Instead of having to slowly diffuse thru the inert gas present, the magnesium vapor will then be rapidly 120 evolved at a sufficient pressure to sweep this gas away and into the condenser; where, by a suitable regulation of the condenser temperature, I continuously condense this vapor in the form of a very pure crystalline 125 mass.

126 It is, of course, necessary that the temperature in the condensing area should be below that of the metal being sublimed, since the difference in vapor pressure due 130

to this difference in temperature is the driving force causing the rapid transfer of the magnesium vapor from the subliming to the condensing end of the system. This difference in pressure must be equal to the sum of the partial pressure of the inert gas present in the condenser and the pressure required to overcome the frictional resistance and force the vapor from the subliming to the condensing end. The importance of these factors is seen by the fact that calculation shows that if magnesium be sublimed in an apparatus such as the one shown in Fig. 1, having a cross-sectional area of one square foot at the section 4-4, at a temperature of 600° C. and a pressure of 0.75 mm., the linear velocity of the magnesium vapor which would be necessary to sublime 100 pounds of magnesium in 24 hours would be in excess of one-half mile a minute. Diffusion, such as would take place if the total pressure within the apparatus were greater than the vapor pressure of magnesium at the temperature employed, is known to take place relatively slowly, and it is evident that my method of sublimation of magnesium will be much more rapid than one which depends upon diffusion. The temperature of sublimation and conversely of solidification may vary from approximately 300 degrees C. at 0.001 mm. pressure to 651 degrees at approximately 2 mm. pressure. The most favorable operating conditions at the present time have been found to be a temperature of approximately 600 degrees C. and a pressure of 0.5-0.2 mm. Under such conditions I am able to sublime 100 pounds of magnesium in 4 hours in an apparatus having a cross section of approximately one square foot.

The crystallized metal can be handled in different ways. It can be placed in an extrusion press and extruded directly into any of the customary structural shapes, such as wire, bars, tubes, rods etc. The crystals can also be compressed into briquets at a temperature of about 200 degrees C. and give a substantially chemically pure metal in a marketable form. This might not be

the case if the metal were first melted and cast, on account of the fact that oxides and nitrides would be introduced into the metal by melting. This metal is also highly resistant to corrosion due to its extreme purity.

I claim:—

1. In a method of producing pure magnesium, the step comprising subjecting material containing metallic magnesium to an absolute pressure less than the vapor pressure of magnesium at its melting point, and heating the said material to its sublimation point to cause the magnesium to vaporize rapidly.

2. The method of producing pure magnesium comprising subjecting material containing metallic magnesium to an absolute pressure less than the vapor pressure of magnesium at its melting point, heating the said material to the sublimation point and thereafter reducing the temperature of the evolved vapor to cause solidification of the magnesium.

3. The method of producing refined magnesium comprising subjecting impure magnesium to such temperature and pressure as will cause the magnesium to sublime rapidly.

4. The method of producing refined magnesium comprising subjecting impure magnesium in a solid form to a temperature not less than about 300 degrees C. and to an absolute pressure less than about 2 mm. of mercury to vaporize the metal and bringing the vapors in contact with a surface, the temperature of which is substantially lower than the melting point of magnesium to cause solidification of the magnesium in the form of crystals.

5. The method of refining impure magnesium comprising subjecting the metal to a temperature between approximately 300 degrees C. and its freezing point and to an absolute pressure of approximately 0.001 to 2 mm.

In testimony whereof I affix my signature.

HERMAN E. BAKKEN.